

## UNITED STATES PATENT OFFICE.

EDGAR RAYMOND CLARK, OF PITTSBURGH, PENNSYLVANIA, ASSIGNOR TO MILTON S. ERLANGER, OF NEW YORK, N. Y.

## COTTON FABRIC HAVING A LINENLIKE FINISH RESISTANT TO WEAR AND WASHING.

No Drawing.

Application filed March 1, 1923. Serial No. 622,223.

*To all whom it may concern:*

Be it known that I, EDGAR RAYMOND CLARK, a citizen of the United States, residing at Pittsburgh, in the county of Allegheny, State of Pennsylvania, have invented certain new and useful Improvements in Cotton Fabrics Having a Linenlike Finish Resistant to Wear and Washing; and I do hereby declare the following to be a full, clear, and exact description of the invention, such as will enable others skilled in the art to which it appertains to make and use the same.

This invention relates to improvements in the treatment of cotton fabrics whereby the treated fabric is given a permanent linen-like appearance and feel, and includes the improved fabric itself as well as the method of its production.

One of the primary objects of the invention is to produce table damask having a linen-like finish, but the invention is applicable to other cotton fabrics where a linen-like finish is desired.

The new fabric of the present invention is a soft, pliable and linen-like fabric, having a linen-like appearance and feel and capable of withstanding repeated laundering. The new fabric has permanently and integrally combined therewith cellulose regenerated from viscose applied to the fabric by a special method of application.

According to the present invention the cotton fabric is treated with a suitable viscose solution, the excess solution removed by pressure, and the viscose then decomposed and cellulose regenerated or precipitated therefrom and in the fibre of the fabric, as more fully hereinafter explained.

The viscose solution employed in the process may be made from cotton rags, linters, cellulose from wood, etc. Bleached cotton linters are well adapted for use. These should be in good chemical condition, that is, free from oxycellulose and other products resulting from the action of chemicals on cellulose, and also free from dirt, oil and leaf or seed particles. In making the viscose solution I keep the alkalinity low

so that the resulting viscose solution will be 50 of medium or low alkalinity, such as is produced for example by using not more than two molecular equivalents of sodium hydroxide to one of cellulose. When inferior forms of cellulose are used in making the 55 viscose solution, the solution may be purified before it is applied to the fabric. By the use of a viscose solution of low alkalinity, and suitably prepared, discoloration 60 of the fabrics is avoided during the drying operation to which they are subjected.

The following specific example illustrates one method of preparing a viscose solution particularly adapted for use in the treatment of cotton fabrics according to the present invention; but it will be understood that the invention is not limited to the preparation of the viscose solution in this particular way, although, as above indicated, the preparation and use of a viscose solution of 65 low alkalinity is of advantage in the practice of the invention; and I consider the production of a viscose solution of low alkalinity in this way to be itself new, and a 70 part of the invention:

100 lbs. of air dry bleached cotton linters, free from dirt, oil, leaf or seed particles, and also free from any of the various products which may result from over-bleaching of such materials, are wet with an excess, say 50 gallons, of caustic soda solution of specific gravity 1.255 at 60° F., containing 20% of sodium hydroxide. The cellulosic material and the caustic soda solution are stirred together for one hour and the mass is then pressed to remove the excess alkali. The pressure is so regulated that the squeezed out mass weighs 350 lbs. This mass is then loosened, spread in open vessels of shallow depth and allowed to age 75 for approximately 24 hours, during which time it should be turned over from time to time to permit of access of air to all the particles. This product is then kneaded with 80 50 lbs. of carbon disulphide in a closed mixer of suitable construction for about 3 hours. The excess solvent is removed by reducing the atmospheric pressure by vac-

uum pumps, and the jelly-like mass is stirred into about 130 gallons of soft cold water. This solution is then cooled to about 40° F. and maintained at that temperature 5 for about 24 hours before use.

The viscose solution produced in this way can advantageously be used in the treatment of cotton fabric in the manner hereinafter described, but it will be understood 10 that the manufacture of viscose by this exact method is not essential.

The treatment of the cotton fabric, according to the present invention, will be further illustrated by describing the treatment 15 of cotton damask with the viscose solution produced in accordance with the above example; but it will be understood that this specific procedure is intended as illustrative of the invention, and that the 20 invention is not limited thereto.

The cotton damask is thoroughly desized and preferably singed, following the usual procedure of bleaching, although the actual 25 bleaching operation may be deferred until after the fabric has been treated with the viscose solution and the permanent finish given to the fabric. Following these preliminary operations, the fabric is brought to a condition of sensible dryness and is then treated on a mangling device in the 30 open width with the viscose solution containing, for example, from 5% to 10% of cellulose. The excess is squeezed out, the pressure being adjusted so that the weight of the fabric is increased about 50%, or in other words so that the permanent increase in weight will be from say 2½% to 5%, depending upon the nature of the goods and the degree of stiffness desired in the product.

The impregnated goods are then carried in a tenting frame, being stretched to the desired finished width, and are made sensibly dry by being subjected to the action of a current of warm dry air, at a temperature 45 not exceeding 120° F., and the length of the frame and conditions of ventilation being properly adjusted to accomplish this result. The goods are then calendered with more or less pressure according to the type 50 of goods being handled and are then without prior washing passed through a bath of dilute sulphuric acid of strength equivalent to say 5% to 10% H<sub>2</sub>SO<sub>4</sub>. The excess acid is then removed by squeezing and rinsing and the goods are then thoroughly cleansed from the difficultly soluble sulphide byproducts which are not of pleasing color by thorough treatment in hot water. Subsequently, the goods may be bleached and finished like ordinary cotton fabrics although starching is not necessary.

In the treatment of the cotton fabric according to the above specific example, it will be seen that the viscose solution is applied to the fabric and the excess solution re-

moved, leaving only such an amount of viscose on and in the fabric as is desired for conversion, by precipitation or decomposition, into cellulose. It will also be seen that the treatment of the fabric with the 70 viscose solution is followed by a drying and calendering operation before the treated fabric is passed through the acid bath for the decomposition of the viscose.

The specific method of procedure, in the treatment of the fabric, may be varied, and other mechanical operations than those mentioned may be employed. For example, the goods may be soaked in the viscose liquor in the rope form, or the drying may be conducted on the can type of drier. So also, other precipitating baths may be used, for the decomposition of the viscose after the calendering operation; for example, baths containing acid or acid salts or combinations thereof, or other materials which precipitate or decompose the viscose. Precipitating solutions may be used of the character used in the manufacture of artificial silk from viscose where the viscose thread or filament is passed into a precipitating bath for converting the viscose into cellulose. The use of a sulphuric acid bath, however, produces a very insoluble deposit and is advantageous for that reason.

It is not necessary to use an after treatment of the fabric with sodium sulphide or other product to clear the fabric, and this is an advantage, since such treatment is injurious to the finish desired.

The treated fabric of the present invention, produced as above described, closely resembles high grade linen damask and other weaves, having a finish which in appearance resembles the ordinary heavy finish produced by the use of starch and softening agents on damasks and other types of cotton fabrics or other highly sized materials, but it is distinguished from such starched or sized fabrics by having a permanent finish which forms a unitary and integral part of the treated fabric and is little damaged, if at all, by repeated washing according to the normal laundering practice in which hot alkaline soap solutions, bleaching solutions, etc., are used. The precipitated viscose is insoluble and is so intimately combined with the cotton fibres that it is substantially unaffected by the mechanical action of laundering or by the common laundering solutions, and remains smooth and flexible even after repeated washings.

The fabric has a smooth finish, but this finish is distinguished from that produced by starching and calendering, since the latter is entirely transient and a single laundering removes it, leaving a loose cotton fabric of ordinary appearance.

The new treated fabric is of high whiteness, has the feel as well as the appearance of

linen, is readily wet by water, flexible, and closely similar in appearance to linen fabrics of equivalent texture. The new fabric is also distinguished from stiff, harsh and impervious fabrics made by treatment with viscose, since the new fabric is soft and pliable and is readily wetted by water and has much the same feel as well as appearance of linen fabric.

10 In the process of the invention, by which the new fabric is produced, it will be seen that a viscose solution of low alkalinity is used, while the drying takes place slowly at a low temperature. The regulation of 15 the alkalinity and temperature, with avoidance of excess alkali and high temperatures, prevents discoloration of the fabric and prevents injuring or tendering the fabric, so that the treated fabric is of superior 20 strength. It will also be seen that the fabric is subjected to a drying and calendering treatment before the acid treatment, with resulting production of a smooth, lustrous and firmly adhering finish. It will further 25 be seen that no sulphides are used after the acid treatment and hence there is no injury to the finish by such use.

The expression "regenerated cellulose" as used in the claims covers cellulose hydrate 30 which has been regenerated from viscose.

I claim:

1. The method of treating cotton fabrics, which comprises impregnating the fabric with a viscose solution of low alkalinity, 35 removing the excess solution and precipitating the cellulose from the viscose by treatment with a precipitating bath.

2. The method of treating cotton fabrics, which comprises impregnating the fabric 40 with viscose of an alkalinity corresponding to less than two moles of caustic alkali to one mole of cellulose, removing the excess solution and precipitating the cellulose from the viscose, substantially as described.

45 3. The method of treating cotton fabrics, which comprises impregnating the fabric with a viscose solution of low alkalinity, removing the excess solution, drying the fabric in a current of warm dry air and precipitating with dilute acid, substantially as described.

4. The method of treating cotton fabrics, which comprises impregnating the fabric with a viscose solution of low alkalinity, removing the excess solution, drying the fabric in a current of warm dry air, precipitating with dilute sulphuric acid, removing excess acid and removing sulfides by treatment with water, substantially as described.

5. The method of treating cotton fabrics, which comprises impregnating the fabric with a viscose solution of low alkalinity, removing the excess solution, drying the fabric in a current of warm dry air, at a temperature not exceeding 120 deg. F.,

and precipitating with dilute acid, substantially as described.

6. The method of treating cotton fabrics, which comprises impregnating the fabric with a viscose solution of low alkalinity, 70 removing the excess solution, drying the fabric in a current of warm dry air, at a temperature not exceeding 120 deg. F., precipitating with diluted sulphuric acid, removing excess acid and removing sulfides by treatment with hot water, substantially as described.

7. The method of treating cotton fabrics, which comprises impregnating the fabric with a viscose solution of low alkalinity, 80 removing the excess solution, drying the fabric in a current of warm dry air, calendering the fabric, and precipitating with dilute acid, substantially as described.

8. The method of treating cotton fabrics, which comprises impregnating the fabric with a viscose solution of low alkalinity, removing the excess solution, drying the fabric in a current of warm dry air at a 90 temperature not exceeding 120 deg. F., calendering and precipitating with dilute sulphuric acid substantially as described.

9. The method of treating cotton fabrics, which comprises impregnating the fabric with a viscose solution of low alkalinity, 95 squeezing out the excess solution to an extent such that the permanent increase in weight of the fabric is about 2½ to 5 per cent, drying the fabric in a current of warm dry air, calendering, precipitating with dilute acid, removing the excess acid and washing out sulfides formed, substantially as described.

10. The method of treating cotton fabrics, which comprises impregnating the fabric with a viscose solution of low alkalinity, containing about 5 to 10 per cent cellulose, 100 squeezing out the excess until there is an increase of weight of about 50 per cent, drying the fabric in a current of warm dry air, calendering, precipitating with dilute sulphuric acid, removing excess acid and washing out the sulfides formed.

11. As a new article of manufacture, a cotton fabric having a permanent washable 115 finish of regenerated cellulose, said fabric being flexible and readily wetted by water and having a linen-like finish and feel.

12. As an article of manufacture, a cotton table damask, having a permanent washable finish of regenerated cellulose, said damask being flexible, readily wetted by water and having a linen-like finish and feel.

13. As a new article of manufacture, a cotton fabric having a permanent washable finish of regenerated cellulose, the amount of said regenerated cellulose being about 2½ to 5% of the weight of the cotton fabric, said fabric being flexible and

readily wetted by water and having a linen-like finish and feel.

14. As an article of manufacture, a cotton table damask, having a permanent washable finish of regenerated cellulose, the amount of said regenerated cellulose being about 2½ to 5% of the weight of the cot-

ton fabric, said damask being flexible, readily wetted by water and having a linen-like finish and feel.

In testimony whereof I affix my signature.

EDGAR RAYMOND CLARK.